

# UNITED STATES PATENT OFFICE.

ARTHUR L. BERRY, OF PORTLAND, MAINE.

## PAINT.

No. 885,973.

Specification of Letters Patent. Patented April 28, 1908.

Application filed January 29, 1908. Serial No. 413,147.

*To all whom it may concern:*

Be it known that I, ARTHUR L. BERRY, a citizen of the United States, and resident of Portland, in the county of Cumberland and State of Maine, have invented new and useful Improvements in Paints, of which the following is a specification:

This invention relates to a paint specially adapted for use upon vessels and it is designed to provide a paint which will tend to preserve the object to which it is applied from decay and from destruction from animals and to prevent the adhesion of any kind of animal or vegetable life.

To this end my invention consists of a paint composed of amorphous graphite, zinc oxide, copper arsenite and turpentine.

It also consists in combining and mixing these in the manner and in about the proportion as hereinafter set forth.

In the manufacture of my improved paint, taking one gallon as the unit, the ingredients are in about the following proportions; amorphous graphite seventy-six ounces, zinc oxide eight ounces, copper arsenite one ounce, and turpentine eighty-eight ounces.

In the manufacture of my improved paint I have found that the best results are obtained by first grinding the amorphous graphite and zinc oxide in turpentine to a pasty consistency. The copper arsenite is then dissolved in sufficient of the turpentine to reduce it to a pasty consistency. The

foregoing products are then ground together in the balance of the turpentine. I find that this produces a slate colored paint which, however, may be changed to any desired color by the addition of suitable coloring matter.

While I have given the proportions which seem to produce the best results, any reasonable variation of these proportions will be within the spirit and scope of my invention.

Having thus described my invention and its use I claim:

1. A paint consisting of amorphous graphite, zinc oxide, copper arsenite and turpentine.
2. A paint composed of amorphous graphite, zinc oxide, copper arsenite and turpentine mixed in about the proportion of 76 oz. graphite, 8 oz. zinc oxide, 1 oz. arsenite and 88 oz. turpentine to the gallon and mixed by grinding the graphite and zinc oxide in turpentine to a pasty consistency, dissolving the arsenite in sufficient turpentine to reduce it to a pasty consistency and then grinding all together in the balance of the turpentine, substantially as described.

In testimony whereof, I have signed my name to this specification in presence of two subscribing witnesses this 27th day of January, 1908.

ARTHUR L. BERRY.

In presence of—

MARIAN RICHARDS,  
LAUREN M. SANBORN.